

Patented Apr. 2, 1940

2,195,419

# UNITED STATES PATENT OFFICE

2,195,419

## PROCESS FOR REDUCING THE DENSITY OF SILVER IMAGES AND COMPOSITIONS THEREFOR

David M. McQueen and Max T. Goebel, Wilmington, Del., assignors to Du Pont Film Manufacturing Corp., New York, N. Y., a corporation of Delaware

No Drawing. Application October 3, 1938,  
Serial No. 233,117

17 Claims. (Cl. 95—88)

This invention relates to photography; more particularly it relates to the processing of light sensitive photographic elements; still more particularly it relates to photographic processes for reducing and/or removing silver images. The invention also relates to processing baths for use in the aforescribed processes.

This invention has for an object new and efficient methods of processing photographic elements. A further object is to provide a rapid and efficient reversal process for treating photographic film. A still further object is to provide an improved process for reducing photographic silver images. A still further object is to modify chemically silver images so that they may be rapidly and completely removed from photographic elements. Still other objects will appear hereinafter.

The above and other objects are accomplished by the following invention which comprises the use of a sulfamic acid in a photographic processing bath. In a more limited sense, they are accomplished by the use of sulfamic acid in conjunction with oxidizing agents for reducing or bleaching silver images. More particularly the invention comprises a photographic bleach bath containing sulfamic acid and an alkali metal or ammonium dichromate or permanganate.

The use of sulfuric acid in conjunction with potassium permanganate or potassium dichromate for reducing or removing silver images has been standard in the art for many years. With potassium permanganate the reaction is probably as follows:



The silver sulfate, being appreciably water-soluble, can be eliminated by washing and, depending upon the time of contact with the bath, the silver image is reduced or completely removed. Procedures of this type have come to be very important in the processing of certain types of films, e. g. sub-standard size motion picture films and certain types of color films. In preparing a direct positive from a negative image by the reversal method, the negative image may be treated with a bath of potassium permanganate or potassium dichromate and sulfuric acid to remove the silver image and the residual silver halide and then re-exposed and developed.

It has now been found that the sulfamic acids, particularly sulfamic acid, can be advantageously used to replace sulfuric acid in a reversal "bleaching" bath and that superior and unexpected results are obtained by such substitution. "Bleaching" as herein used refers to a process by which silver is converted to a silver salt which is usually an appreciably water soluble salt which is thereupon removed from the photographic film. It

has been found that the silver sulfamates, particularly silver sulfamate, are exceedingly more soluble in the usual photographic and washing baths. This increased solubility is a distinct advantage since it means that silver images may be more completely removed. The action of bleach baths containing a sulfamic acid, particularly sulfamic acid, furthermore, have been found to be more rapid than the sulfuric acid which is usually employed.

The invention will be further illustrated but is not to be limited by the following examples in which the parts stated are parts by weight:

### Example I

A negative motion picture film was exposed and given the following treatments:

(1) Development for 8-9 minutes in a developer of the following composition:

|                          | Parts |
|--------------------------|-------|
| Water                    | 1000  |
| Metol                    | 1.5   |
| Hydroquinone             | 1.5   |
| Anhydrous sodium sulfite | 8.0   |
| Potassium thiocyanate    | 3.0   |
| Potassium bromide        | 3.0   |
| Potassium carbonate      | 20.0  |

(2) Five minutes washing in running water

(3) Bleaching for 3-4 minutes in a bath of the following composition:

|                      | Parts |
|----------------------|-------|
| Water                | 1000  |
| Potassium dichromate | 4.5   |

Sulfamic acid

35

(4) Washing in running water for 5 minutes;

(5) Clearing for 5 minutes in a bath of the following composition:

|                  | Parts |
|------------------|-------|
| Water            | 1000  |
| Sodium bisulfite | 20    |

40

(6) Washing for 8 minutes in running water;

(7) Exposure to strong artificial light;

(8) Development for 6 minutes in a bath of the following composition:

|                          | Parts |
|--------------------------|-------|
| Water                    | 1000  |
| Metol                    | 1     |
| Hydroquinone             | 6     |
| Anhydrous sodium sulfite | 25    |
| Potassium bromide        | 1     |
| Potassium carbonate      | 40    |

50

(9) Washing for ten minutes in running water.

By this procedure a positive of excellent quality was obtained. Step (5) may sometimes be omitted.

### Example II

A negative motion picture film was exposed and then given the following treatments:

(1) Development for approximately 5 minutes at 18° C. in a bath of the following composition:

|                                   | Parts |
|-----------------------------------|-------|
| 5 Water                           | 4500  |
| 5 Metol                           | 13    |
| Anhydrous sodium sulfite          | 100   |
| Potassium bromide                 | 5.5   |
| Ammonium hydroxide (sp. gr. 0.90) | 27    |
| Hydroquinone                      | 4     |

10 (2) Washing for 5-10 minutes in running water;

(3) Bleaching for 3 minutes at 18° C. in a bath of the following composition:

|                      | Parts |
|----------------------|-------|
| 15 Water             | 1325  |
| Sulfamic acid        | 17.5  |
| Potassium dichromate | 3     |

(4) Washing for 5 minutes in running water;

20 (5) Clearing for 6 minutes in a bath of the following composition:

|                          | Parts |
|--------------------------|-------|
| Water                    | 1000  |
| Anhydrous sodium sulfite | 100   |

25 (6) Washing for 8 minutes in running water;

(7) Exposure to diffuse daylight for one minute;

(8) Development for 5 minutes at 18° C. in a bath of the following composition:

|                          | Parts |
|--------------------------|-------|
| Water                    | 1000  |
| Metol                    | 2     |
| Hydroquinone             | 4     |
| Anhydrous sodium sulfite | 25    |
| Sodium carbonate         | 18.5  |
| Potassium bromide        | 2     |

(9) Washing for ten minutes in running water.

By this procedure a very clean positive of 40 excellent gradation was obtained.

### Example III

A color film of the ruled screen type was exposed and processed as follows in total darkness:

45 (1) Development for 4 minutes in a bath of the following composition

|                       | Parts |
|-----------------------|-------|
| 50 Metol              | 6.5   |
| Hydroquinone          | 1.25  |
| Sodium sulfite        | 100   |
| Sodium carbonate      | 95    |
| Potassium bromide     | 2.75  |
| Potassium thiocyanate | 9     |
| 55 Water              | 790   |

(2) Treatment for 2 minutes in a 1% solution of acetic acid;

(3) Washing for 5-10 minutes in running water;

60 (4) Bleaching in a bath of the following composition

|                        | Parts |
|------------------------|-------|
| Potassium permanganate | 2     |
| Sulfamic acid          | 15    |

65 Water

1000

(5) Washing for 5-10 minutes in running water;

(6) Clearing in a 2.5% solution of potassium metabisulfite;

70 (7) Washing in running water for 2 minutes;

(8) Exposure for 3-4 minutes to a 100 watt lamp at a distance of 3 feet;

(9) Development for 6 minutes in the original developer;

(10) Washing in running water for 4 minutes;

(11) Treatment for 2 minutes with a 40% solution of sodium thiosulfate;

(12) Washing in running water for 15 minutes. By this procedure an excellent color transparency of good detail and color contrast was obtained.

### Example IV

A negative was made by exposing a multilayer film, that is, a film coated with emulsions of different spectral sensitivities as is common in certain processes of color photography. In this case the film was composed of a panchromatic emulsion deficient in green sensitivity coated over cellulose acetate base, a clear gelatin layer, an orthochromatic emulsion, a layer of gelatin dyed yellow and, on top, a layer of emulsion sensitive only to blue and ultraviolet light. This was developed in a metol-hydroquinone developer and thoroughly washed. The silver deposits were then bleached with a bath of the following composition:

|                      | Parts |
|----------------------|-------|
| Water                | 1000  |
| Potassium dichromate | 6     |
| Sulfamic acid        | 20    |

and cleared in a bath of two per cent sodium bisulfite solution.

The silver was found to be removed completely and no stain was left in the film. This film is suitable for further processing to pictures in color, as described in the art.

In place of sulfamic acid itself which is described in the specific examples, other sulfamic acids may be substituted. However, it is to be distinctly understood that sulfamic acid is the prepared reagent and has superior photographic properties. As examples of suitable acids, mention is made of the lower mono- and di-alkyl sulfamic acids, e. g. mono-methyl-sulfamic acid, mono-ethyl-sulfamic acid, di-methylsulfamic acid, di-ethylsulfamic acid; methylolsulfamic acid, etc. The easily hydrolyzable salts, e. g. aluminum sulfamate may also be used.

The sulfamic acids may be incorporated in the bath over a fairly wide range of proportions. For instance, 2 to 30 grams of sulfamic acid per liter of water represents a practical range and 5 to 10 grams per liter a preferred range. Similar amounts of the substituted sulfamic acids may be used.

The amount of oxidizing agent used may likewise vary over a fairly wide range. For instance from 25 to 2 grams per liter of potassium dichromate or potassium permanganate represents a practical range and 10 to 2 represents a preferred range. Similar amounts of other oxidizing agents may be used.

In place of the oxidizing agents set forth in the preceding examples, any oxidizing agent which will aid in solubilizing the silver so that it will form a sulfamic acid salt and which does not destroy the sulfamic acid used may be substituted for those set forth in the examples. The oxidizing agents preferably should not have an adverse effect on the gelatin binder. As examples of other utilizable oxidizing agents, mention is made of ferric ammonium sulfate, ceric ammonium sulfate, ammonium persulfate, sodium dichromate sodium permanganate, ammonium dichromate and ammonium permanganate. Mixtures of the above-described agents including those of the examples may be used. The alkali metal dichro-

mates and permanganates give the best results and represent the preferred embodiment hereof.

The processing baths of the present invention comprising in its preferred form sulfamic acid and potassium dichromate or potassium permanganate are not limited in their use to reversal bleaching processes but may be used in various types of processes wherein a photographic reducer is required. Thus, if the concentration of sulfamic acid and oxidizing agent is materially reduced, the resulting bath may be used to lessen the density of films containing silver images. The period of processing is generally less than that required for a reversal procedure.

The baths may be used with practically any type of photographic element containing a silver image. For instance, they may be used in conjunction with motion picture film, either for color or black and white photography, still camera films or plates, "permanent record" film suitable for the use of recording business, library and historical documents, and non-motion picture film which is sometimes processed by reversal in order to obtain fine grain. They may also be used in conjunction with direct paper print cameras and copying machines.

The use of the "bleaching baths" of the present invention, furthermore, is not to be limited by the other steps set forth in the examples. For instance, any normal type of developer may be used, and the exposure after bleaching may be controlled or carried to complete blackening.

The "bleaching" baths of the present invention may contain besides the above-mentioned constituents, other agents, such as materials added to decrease the penetration of the bath, such as alcohol, acetone and glucose; softening agents for the photographic film and emulsion, such as glycerol; hardening agents, e. g. inorganic salts with no specific effect on silver images or silver halides.

The removal of silver from photographic films has been found desirable in a number of methods of processing. As hereinbefore mentioned, the customary procedure has been to employ a bath of oxidizing agent which has no deleterious action on the gelatin of the emulsion, and sulfuric acid. Attempts to supplant sulfuric acid have not been successful, and its use has become more or less standard in the industry. Thus, replacement by nitric acid, the silver salts of which are more soluble in water than silver sulfate has not proven to be successful. Acetic acid has been proposed but is not satisfactory for a number of economic reasons, including the fact that its slow speed renders it practically useless.

It therefore could not be predicted from the acids just described that the sulfamic acids, particularly sulfamic acid, could be advantageously used in conjunction with certain oxidizing agents to remove silver. Silver images are removed rapidly and completely by the use of such acids. This is an economic advantage in that it saves valuable processing time. A further advantage resides in the fact that less processing equipment such as washing equipment in continuous processes is required. Furthermore, the use of sulfamic acid leads to cleaner films and results in finer picture detail.

Since sulfamic acid is a nonhygroscopic, crystalline solid its use presents marked advantages in convenience of handling as compared with sulfuric and other acids. It can be readily weighed out without special precautions and furthermore does not present the corrosive hazard involved

in the use of sulfuric acid. It possesses the properties of a strong acid. A novel method for preparing this acid, thus rendering it available for the present process, has been described in U. S. Patent 2,102,350.

The use of the sulfamic acids, particularly sulfamic acid, in bleaching is especially advantageous in the processing of color films, particularly those of the multilayer type, where removal of the silver after the first development is very often difficult and incomplete. The use of these acids as bleaching agents results in increased color contrast of the finished pictures and in an improvement in definition which is of great importance in color work. The outstanding rapidity of action of baths comprising sulfamic acid and an oxidizing agent is also peculiarly suited for use with films which demand rapid processing, as for example, in the processing of records of business documents, checks, etc.

As many apparently widely different embodiments of this invention may be made without departing from the spirit and scope thereof, it is to be understood that we do not limit ourselves to the specific embodiments herein except as defined by the appended claims.

We claim:

1. An aqueous photographic bleach bath comprising an oxidizing agent and a compound taken from the group consisting of sulfamic acids and their easily hydrolyzable salts.

2. An aqueous photographic processing bath containing a sulfamic acid and an oxidizing agent.

3. A photographic processing bath comprising an aqueous solution containing sulfamic acid and an oxidizing agent.

4. A photographic bleach bath comprising an aqueous solution containing from 0.2 to 3% of sulfamic acid and 2.5 to 0.2% of an oxidizing agent.

5. A photographic bleach bath comprising an aqueous solution containing sulfamic acid and an alkali metal dichromate.

6. A photographic bleach bath comprising an aqueous solution containing sulfamic acid and ammonium persulfate.

7. A photographic bleach bath comprising an aqueous solution containing sulfamic acid and an alkali metal permanganate.

8. A process for reducing the opacity of a silver deposit which comprises treating the same in an aqueous processing bath containing a sulfamic acid and an oxidizing agent.

9. A process which comprises reducing the density of the silver image of a photographic element by treating the latter in an aqueous bath containing an oxidizing agent and a compound taken from the group consisting of sulfamic acids and their easily hydrolyzable salts.

10. A process which comprises reducing the density of the silver image of a photographic element by treating the latter in an aqueous bath containing a sulfamic acid and an oxidizing agent.

11. A process which comprises reducing the density of the silver image of a photographic element by treating the latter in an aqueous bath containing sulfamic acid and an oxidizing agent.

12. In a process of producing positives by a reversal method the step which comprises treating a photographic element containing a silver image with an aqueous bath containing a sulfamic acid and an oxidizing agent.

13. In a process of producing positives by a

reversal method the step which comprises treating a photographic element containing a silver image with an aqueous bath containing sulfamic acid and an oxidizing agent.

14. A photographic reversal process comprising exposure to an image, development in an ordinary photographic developer, bleaching in a processing bath containing sulfamic acid and an oxidizing agent and development of the reversed image.

15. A photographic reversal process comprising exposure to an image, development in an ordinary photographic developer, bleaching in a processing bath containing sulfamic acid and an oxidizing agent, re-exposure to light, and development of the reversed image.

16. A photographic reversal process comprising exposure to an image, development in an ordinary photographic developer, bleaching in a processing bath containing sulfamic acid and an oxidizing agent and processing the reversed image to pictures in color. 5

17. A photographic reversal process comprising exposing a multilayer film coated with emulsions of different sensitivity, developing the latent images in an ordinary photographic developer, bleaching the developed film in a processing bath containing sulfamic acid and an oxidizing agent and processing the reversed images to pictures in color. 10

DAVID M. McQUEEN. 15  
MAX T. GOEBEL.